

Aug. 9, 1949.

A. L. J. QUENEAU

2,478,594

## METHOD OF CONDENSING ZINC

Filed Aug. 13, 1947



INVENTOR  
AUGUSTIN L. J. QUENEAU

BY  
Pennis, Edmunds, Norton and Barrows  
ATTORNEYS

## UNITED STATES PATENT OFFICE

2,478,594

## METHOD OF CONDENSING ZINC

Augustin L. J. Queneau, Morristown, N.J.

Application August 13, 1947, Serial No. 768,392

7 Claims. (Cl. 75—88)

1

This invention relates to the recovery of zinc from its ores, and more particularly to improvements in the method of and apparatus for condensing zinc vapor from the furnace in which the ore is smelted.

The gases and vapors which are released in the smelting of zinc carry large quantities of both sensible and latent heat. The temperature of the gases and vapors is of the order of 950°—1000° C., and the zinc is in the form of vapor from which the latent heat of vaporization must be withdrawn in order to effect the condensation. The metal must also be cooled to the desired temperature. Thus, one of the major problems of the zinc industry for many years has been the efficient condensation of zinc vapors and the separation of the zinc from the inert gases such as nitrogen and carbon monoxide which accompany the zinc vapors.

It is the object of the present invention to provide a simple, effective and economical method of condensing and separating zinc from the smelter gases and vapors.

Another object of the invention is the provision of apparatus in which the method may be conducted in an economical and efficient manner.

Other objects and advantages of the invention will be apparent as it is better understood by reference to the following specification and the accompanying drawing, which illustrates diagrammatically an apparatus adapted to permit accomplishment of the stated objects.

The invention depends upon the use of molten zinc as a coolant for the gases and vapors released from the smelting furnace, and the circulation of large quantities of such molten zinc for that purpose. In carrying out the invention, molten zinc from a holding furnace is circulated continuously to and from a condenser in which the zinc is distributed in dispersed form for maximum contact with the gases and vapors which are cooled rapidly from the high temperature at which they enter the condenser to a temperature of about 500°—525° C., and in any event to a temperature above the freezing point of zinc, 420° C.

Owing to the pressure exerted by the gases and vapors from the smelting furnace, for example about five pounds per square inch, the inert or fixed gases, nitrogen, carbon monoxide, etc., are forced through the pool of molten zinc at the bottom of the condenser as bubbles, thus assuring condensation of any remaining zinc vapor. These gases eventually leave the molten zinc which flows into the holding furnace. The gases may be treated thereafter to recover any zinc

2

oxide, blue powder or the like. The latter can be returned for reprocessing and introduction to the smelting furnace to recover the zinc content. The gases, free from zinc products, may be compressed and used for any desirable purpose, or discarded to the atmosphere. The zinc collected in the holding furnace is recirculated and from time to time the excess resulting from condensation of the zinc vapor is pumped from the furnace and cast or molded.

The procedure as briefly outlined ensures the maximum recovery of zinc vapors as metallic zinc and the minimum of zinc oxide, blue powder and the like. The molten zinc is readily maintained and circulated to act as a coolant in the condenser, and is the most efficient coolant for that purpose. All of the zinc content of the furnace gases and vapors is eventually recovered. The operation is efficient and economical, and a substantial improvement in the methods heretofore available.

The procedure will be better understood by reference to the accompanying drawing, in which 5 indicates a smelting furnace, for example a blast furnace adapted to be supplied with a dry blast of oxygen-enriched air through a pipe 6 connected to tuyères 7. As the result of the smelting operation, gases and vapors are delivered through a pipe 8 at a temperature in the neighborhood of 950°—1000° C. It is desirable to maintain the gases at this temperature to avoid the possibility of a reversible reaction in which carbon monoxide is broken down into carbon dioxide and carbon. The presence of carbon dioxide is undesirable, 35 since it reacts with zinc to produce zinc oxide and carbon monoxide.

The pipe 8 delivers the gases and vapors to a condenser 9 consisting of a steel shell lined with a suitable refractory material such as carbon, carbon or graphite. The pipe 8 is similarly lined. The condenser is provided with manholes closed by covers 10 and 11 to permit inspection of the interior of the condenser. Within the condenser, a block 12 of graphite is provided with a central opening 13 and a plurality of upwardly directed passages 14. The central opening 13 is connected by a pipe 15 of graphite or similar material to a pump 16 submerged in molten zinc in a holding furnace 17. The pump 16 may be constructed of graphite or like material in accordance with the disclosure of my application Ser. No. 757,404, filed June 27, 1947. The pump 16 permits the circulation of molten zinc from the holding furnace through the pipe 15 to the distributor 12. Thus the molten zinc is delivered

to the condenser 9 in dispersed form, that is in a spray or rain of fine particles which fall through the atmosphere of the condenser and wash the walls thereof. The molten zinc is thus brought into intimate contact with the gases and vapors entering through the pipe 8, and the zinc vapors are rapidly condensed and cooled to the desired temperature, that is, preferably between 500° and 525° C.

Since there is a large amount of surplus heat, 10 water is sprayed continuously on the wall of the condenser by means of a plurality of pipes 18 in quantity sufficient to maintain satisfactory temperature conditions in the condenser.

A large pool of molten zinc 19 accumulates in the bottom of the condenser. This pool is sufficient in amount to fill a connection 20 between the upwardly-directed leg 9 and a second upwardly-directed leg 21 of the condenser, and extends upward into the leg 21, where the molten zinc is supported by the pressure of the gases within the condenser. The connection 20 is cooled by sprays of water directed thereon through pipes 22. The connection 20 and leg 21 are preferably lined with the same material used as a lining for the condenser 9. Such material has a high heat conductivity, thus permitting energetic cooling by the water sprays.

A pipe 23 of graphite or similar material is connected to the leg 21 and to a downwardly extending pipe 24. The molten zinc which accumulates in the condenser 9 is forced over by the pressure of the gases into the pipes 23 and 24, and thus is delivered to the pool of molten zinc 25 in the holding furnace 17. A refractory cover 26 is provided on the end of the pipe 23 to permit inspection of the interior of the pipe through the manhole in a wall of the holding furnace 17 which is normally closed by a cover 27. A pump 28, similar to the pump 16, is connected to a pipe 29 of graphite or similar material, through which the molten zinc can be withdrawn from time to time and delivered to a mold or casting machine 30.

A pipe 31 extends above the pipe 23 and above the level indicated at 32 is preferably lined with firebrick in order to conserve the heat in the molten zinc which splashes upwardly during the evolution of the gases therefrom. Above the pipe 31, a pipe 33 extends upwardly. It need not be lined, because at this level the temperature of the gases has dropped to 400° C. or less. A pipe 34 delivers the gases to a wet scrubber 35, preferably of the Theisen or Bian type, in which any remaining zinc vapor is separated from the gases in the form of blue powder or zinc oxide. This material, together with the water used in the scrubber, is delivered through a pipe 36 to a settler 37 in which the zinc oxide and blue powder collect. The surplus water is withdrawn through a pipe 38 to a collector 39 and may be re-used.

The gases, freed from practically all of the zinc products, are delivered through a pipe 40 to a baghouse 41 which may be of the usual type, preferably with shaking mechanism for the bags. Any remaining zinc oxide or blue powder is filtered from the gases and collected. This material, together with the solids from the settler 37, may be reprocessed and returned to the smelting furnace in order to recover the zinc content.

The gases escape through a pipe 42 and, being still at a relatively high temperature, are passed through an exchanger 43 which is cooled by water supplied through pipes 44. After cooling, the gases are delivered by a pipe 45 to a compressor

46 and thence through a pipe 47 to a gas holder 48. The gases may be withdrawn as required through a pipe 49 for use, or they may be discharged to the atmosphere.

5 In starting the operation, it is necessary to have the zinc in the holding furnace in a molten condition and also to maintain the pipe 15 at a proper temperature. A burner 50 is disposed in the wall of the holding furnace 17 and is adapted to burn oil, gas or other material in order to raise the temperature of the furnace to the desired point. An electric heating coil 51 may be disposed about the pipe 15 externally of the furnace 17 so that the pipe is sufficiently heated to prevent freezing of the molten zinc therein.

20 In the operation of the device, it is necessary to circulate relatively large quantities of molten zinc at a temperature preferably between 500° and 525° C. The rate of circulation should be 10-30 times the hourly production of zinc vapor in the smelting furnace. Thus, if the blast furnace rate of production is two and one-half tons of zinc vapor per hour, the molten zinc injected into the condenser would be supplied at a rate varying between 25 and 75 tons per hour, the quantity varying with the temperature and relative proportions of zinc vapor and gases issuing from the furnace.

25 The zinc holding furnace may have a capacity of 135-150 tons in order to supply the required metal for circulation through the condenser. The incoming gases, after dropping the zinc vapor as a result of contact with the dispersed molten zinc, are forced to bubble through the molten zinc 30 in the pool at the bottom of the condenser and in the legs 20 and 21. The circulating zinc and the condensed zinc pass through the vertical leg 21 in a series of surges or spouts, under sufficient positive pressure to overcome the head of molten zinc in the leg 21. The length of this leg is such that the zinc rises to a point where it overflows 35 through the pipe 23 into the holding furnace.

40 The uncondensed gases, substantially zinc-free with the exception of zinc vapor saturating these gases at their temperature and pressure, continue upwardly for treatment in the scrubber and baghouse as hereinbefore described.

45 Various changes may be made in the procedure as described and in the apparatus employed therein without departing from the invention or sacrificing the advantages thereof.

I claim:

1. The method of condensing zinc from gases and vapors produced in a smelting furnace which comprises spraying molten zinc in finely-divided form into the upper portion of one leg of a condenser having two upwardly-directed legs connected at their lower portions from a spray nozzle positioned in the upper portion of said one leg, introducing the gases and vapors from the furnace into said one leg of the condenser for intimate contact with the molten zinc sprayed therein with resultant condensation of zinc from said vapors, maintaining a sufficient body of molten zinc in the lower portion of the condenser to maintain the connection between the two legs thereof full of molten zinc, maintaining the gases and vapors in said one leg of the condenser under a pressure sufficient to force molten zinc of said body upwardly into the other leg of the condenser and to force gases and vapors from which zinc was condensed through said connection and upwardly through the molten zinc in said other leg, removing the gases passing upwardly through the molten zinc in said other leg

from said other leg, recovering the residue of zinc oxide and blue powder from said removed gases, and withdrawing molten zinc from the condenser.

2. The method of condensing zinc from gases and vapors as set forth in claim 1 in which the gases and vapors in said one leg of the condenser are maintained under a pressure of about 5 pounds per square inch.

3. The method of condensing zinc from gases and vapors as set forth in claim 1 in which the molten zinc sprayed into the upper portion of said one leg of the condenser is at a temperature of from about 500° C. to 525° C.

4. The method of condensing zinc from gases and vapors as set forth in claim 3 in which the temperature of the gases and vapors introduced into said one leg of the condenser is between about 950° C. and 1000° C.

5. The method of condensing zinc from gases and vapors as set forth in claim 1 in which molten zinc withdrawn from the condenser is recirculated and is sprayed into the upper portion of said one leg of the condenser.

6. The method of condensing zinc from gases and vapors as set forth in claim 1 in which the molten zinc sprayed into the upper portion of

said one leg of the condenser is at a temperature from about 500° C. to 525° C. and the gases and vapors in said one leg of the condenser are maintained under a pressure of about 5 pounds per square inch.

7. The method of condensing zinc from gases and vapors as set forth in claim 6 in which the temperature of the gases and vapors introduced into said one leg of the condenser is between about 950° C. and 1000° C.

AUGUSTIN L. J. QUENEAU.

REFERENCES CITED

15. The following references are of record in the file of this patent:

UNITED STATES PATENTS

| Number       | Name             | Date          |
|--------------|------------------|---------------|
| 20 1,966,627 | Johannsen et al. | July 17, 1934 |
| 2,070,101    | Weaton et al.    | Feb. 9, 1937  |
| 2,208,586    | Kemmer           | July 23, 1940 |
| 2,238,819    | Neve             | Apr. 15, 1941 |
| 2,348,194    | Crane et al.     | May 9, 1944   |
| 25 2,381,403 | Chisholm         | Aug. 7, 1945  |
| 2,381,405    | Griswold, Jr.    | Aug. 7, 1945  |